

F. H. RICHARDS.

ART OF MAKING TYPES AND TYPE BAES.

APPLICATION FILED JAN. 3, 1901. RENEWED JAN. 14, 1909.

919,232.

Patented Apr. 20, 1909.

2 SHEETS—SHEET 1.

Fig. 1.

U.S. PATENT OFFICE

Fig. 2. b



Fig. 3.



Fig. 4.



Fig. 5. Fig. 6.



Fig. 7.



Fig. 8.



Witnesses:

C. W. Smith

T. H. Thompson.

Inventor:

F. H. Richards.

F. H. RICHARDS.

ART OF MAKING TYPES AND TYPE BARS.

APPLICATION FILED JAN. 3, 1901. RENEWED JAN. 14, 1909.

919,232.

Patented Apr. 20, 1909.

2 SHEETS—SHEET 2.

Fig. 9.



Witnesses:

C. W. Smith

J. H. Chapman

Inventor:

F. H. Richards

# UNITED STATES PATENT OFFICE.

FRANCIS H. RICHARDS, OF HARTFORD, CONNECTICUT, ASSIGNOR, BY MESNE ASSIGNMENTS,  
TO AMERICAN TYPOGRAPHIC CORPORATION, A CORPORATION OF NEW JERSEY.

## ART OF MAKING TYPES AND TYPE-BARS.

No. 919,282.

Specification of Letters Patent.

Patented April 20, 1909.

Application filed January 3, 1901, Serial No. 41,935. Renewed January 14, 1909. Serial No. 472,296.

*To all whom it may concern:*

Be it known that I, FRANCIS H. RICHARDS, a citizen of the United States, residing at Hartford, in the county of Hartford and 5 State of Connecticut, have invented certain new and useful Improvements in the Art of Making Types and Type-Bars, of which the following is a specification.

This invention relates to the art of making 10 types and typebars, and especially to a method of making from a solid blank or bar of metal a typebar adapted for use in the typographic art for printing a line of characters.

15 The present invention is in the nature of an improvement upon that shown, described, and claimed in the application of Darien W. Dodson, Serial No. 600,152, filed July 22, 1896, to which I have permission to refer, 20 and also is an improvement upon the invention set forth in my prior application Serial No. 740,512, filed December 16, 1899. In the Dodson process the separate types are formed on the edge of a typebar-blank by 25 a rolling movement of the dies. This rolling movement, however, in the Dodson process, is a simple one, it being a progressive cycloidal movement in a proper orbit.

Two of the principal features that dis- 30 tinguish the present process and the process set forth and claimed in my aforesaid prior application from that of Dodson are these: I avoid the necessity of setting off the finished type-blank before the die is brought 35 into action, and I preferably subject each type-formative portion of the blank to repeated rolling operations usually of such a character that not only will the face of the type be perfectly finished, but the base portion will also be finished and strengthened 40 to such an extent as to enable it to resist greater crushing forces and last longer.

In my prior application hereinbefore referred to I have set forth and claimed a 45 method of forming a type by subjecting a type-blank to repeated type-forming operations, preferably by rolling the type-blank in contact with a type-die, to shape the type gradually, the type-forming operation 50 proceeding in such a manner that most of the surplus stock will be forced out sidewise of a typebar-blank when the type is formed on the edge of such a blank, instead of being forced out endwise thereof as in the Dodson 55 process.

As to one feature thereof the present invention is not only in the nature of an improvement upon, but is also a modification of, that disclosed in my aforesaid application; but as to other features thereof the 60 present invention is entirely distinct from that disclosed in said application, and the actions hereinafter to be described may result from other modes of operation than that set forth in such prior case. 65

The principal feature of the present invention is the formation of a type from a type-blank or from a typebar-blank by working a suitable portion of the type-blank or typebar-blank at such a high rate of speed that the 70 molecular action in the mass will be increased mechanically to such an extent as to result in increasing the ductility of the metal and preferably so softening it as to permit the shaping of the type-face substantially by a 75 molding operation. This heating up of the mass to be shaped by a die is due entirely to the rapid shifting of the mass as a suitable force is applied thereto for shifting or working the same, and the resultant localization 80 of the heat, due to the fact that it is not conducted away or otherwise dissipated as fast as it is developed; and provided that the metal be worked with sufficient rapidity to bring about the proper molecular action and 85 raise the temperature of the mass to a point where it can be shaped more readily, the particular means for working such metal is not essential. I deem it desirable, however, to operate upon the metal of the blank in sub- 90 stantially the manner described in my application hereinbefore mentioned, that is to say, I prefer to roll the metal of the blank repeat- 95 edly in contact with a die, for the purpose of gradually shaping the blank into the form of a type by a series of operations which coact to finish the type perfectly and also to strengthen the body of the type very materi- 100 ally during the shaping thereof. In the pres- ent case, however, when the blank is rolled in contact with a die the rate of operation should be very much higher than when a type is formed according to the process disclosed in my aforesaid application. Usually one of these two coöperating members—viz., 105 the die and the type-blank—will be recipro- cated in a curvilinear path while in contact with the other, and a feed movement will also be imparted to one of them in a direc- 110 tion toward the other, but such reciprocatory

curvilinear movement should be so rapid as to modify the process disclosed in my aforesaid application by adding to the rolling, swaging, and forging operations resulting from the movement of one of said parts in contact with the other while the metal of the blank is substantially unchanged as to its physical state, the additional operation of molding the face of the type, and other portions thereof, after the metal has been properly softened by the heat developed by the rapid mechanical working of the blank.

In the drawings accompanying this specification and forming part of the present application, Figures 1 and 2 are, respectively, a plan and a side elevation of a typebar made by my improved process and enlarged about one-half. Fig. 3 is a plan of a portion of a partially-finished bar enlarged to about five times the natural size, and illustrates the appearance of finished and partly-finished types on the edge of a typebar-blank. Fig. 4 is a sectional side elevation of one end of the same, illustrating the operation of a die for forming a character. Figs. 5 and 6 are sectional end elevations illustrating, respectively, an intermediate and the final stage of the operation of forming a type. Fig. 7 is a side elevation of a die-wheel and a blank-feeding wedge coöperative with a typebar-blank, the parts being shown on the same scale as in Figs. 1 and 2. Fig. 8 is an end view of Fig. 7; and Fig. 9 is a sectional elevation of a simple mechanism for forming types and typebars according to my present process.

Similar characters designate like parts in the different figures of the drawings.

In order to obtain the best results in carrying out my improved process it has been found advantageous, although, of course, it is not absolutely necessary, to form each type by means of a single tool or die coacting with a proper blank, and to so operate one or both of these members relatively to the other or to each other as to compact and condense most perfectly the material of the type proper before the completion of the same. The many experiments that were made to determine the best method of forming types and typebars from blanks demonstrated that it was desirable to condense the metal of the finished type as much as possible both at the face of the type and near the base thereof, and it was also found that the die filled most perfectly when the blank was composed of a plurality of metals having different properties, which metals when alloyed would form a hard and tough compound that would oppose considerable resistance to the action of a type-forming die and yet have sufficient ductility to be worked readily into shape, especially when subjected to repeated rollings by a die for the purpose of gradually forming a type. It was also found that when this gradual formation of a type was effected by

moving one of the two coacting members—viz., the blank and the die—in contact with the other at a high rate of speed the type-forming operation would be finished more quickly and that the rapid formation of the type would be facilitated by the heat developed as a result of the increased molecular action due to the mechanical shifting in position, or working, of the particles of the metal subjected to the type-forming action. For example, when this process was carried out by oscillating the blank at the rate of two thousand or more oscillations per minute, and this blank was an alloy consisting of tin, antimony, and copper combined in suitable proportions for the purpose of obtaining a very hard and tough type-metal, the heat developed by the working of the metal in contact with the die was sufficient to heat the type-metal in the die-space to the point of softening, when there would be added to the type-forming operations of rolling, swaging, and forging the additional operation of molding the heated or softened surface of the metal in contact with the walls of the die while the metal immediately below the softened portion retained its solidity and its capacity to resist the forging, swaging, rolling, and molding operations exerted upon the mass being worked. It should be understood, of course, that the exact rate of speed at which the operation is carried on will vary considerably in practice according to the composition of the type-metal, the extent of the movement of the part operated, &c., and in some cases when the blank is oscillated in the manner just stated, the number of oscillations per minute may reach four to six thousand and upward.

The heating up of the metal or type-blank which is to form the type may be effected in any suitable manner, but while hand-operated means may be employed for the purpose, suitable mechanism will ordinarily be used. Moreover, a single die will usually be employed for operating upon each separate face of a type-block or type-blank, for the reason that such a die is sufficient to subject said type-blank to all of the various operations which it undergoes before becoming a finished type. Any proper type-die may be employed, and this may be mounted in any desired manner, though I prefer to support one or more type-dies, such as *d*, on a carrier, such as *D*, which carrier may be secured to a shaft, such as *Z*, (see Figs. 7 and 8.)

The blank, which may be of any material suitable for the purpose, but will usually be a type-metal of proper composition, is designated herein in a general way by *b*, and may be supported by a carrier substantially in the manner shown in Fig. 9, in which I have illustrated an organized mechanism embodying the elements illustrated diagrammatically in Fig. 7. In said mechanism the typebar-

blank *b* is supported by a carrier, or carriage, which may be of the type illustrated at *B*, and is preferably mounted for traveling movement on a suitable base or support, 5 such as *1'*, forming part of a frame, such as *1*, for supporting the several parts of the mechanism, said carriage here deriving its traveling movements from a feed-screw, such as *20*, which may be turned different distances to 10 feed the carriage correspondingly. In the present construction this carriage also supports a vertically-movable carrier *B'*, which is mounted in guideways in the carriage *B* for the purpose of feeding the blank toward 15 the die during the type-forming operation. Moreover, said vertical carrier is also intended to support another carrier such as *B''*, which constitutes the blank-carrier proper and is preferably mounted for oscillation in bearings in the carrier *B'* by means 20 of trunnions, such as *3*, the axis of oscillation of the carrier *B''* being preferably in the central, vertical, longitudinal plane of the blank *b* when the latter is in place in said carrier. 25 The die-carrier *D*, with which the blank-carriers are intended to coöperate, preferably has its shaft *2* journaled in a bearing in the upper end of an upright *1''* rising from the base *1'*, and said carrier may be turned to any 30 desired position and then held in place in such position by a suitable locking device, such as a spring-pressed detent-pin *12*, carried in this case by an arm *2'* projecting from the bearing for the shaft *2*, said detent-pin 35 being intended to be received in openings, such as *13*, in the die-carrier *D*, for the purpose of holding the die-carrier in the desired working position. Said die-carrier may have a complete series of dies, one for each letter 40 of the alphabet, as clearly shown in Fig. 9. For the purpose of operating one of the main coacting members—viz., the blank and the die—relatively to the other at a high rate of speed, and feeding one of said members to 45 ward the other during such rapid type-forming movement, I have illustrated herein a main driving-shaft *15*, carrying in this case a pair of pulleys, one of which is designated by *15'* and is driven at a high rate of speed by a 50 driving-band *16* from some suitable source of power, (not shown,) while the other transmits its movement to a driving-band *17*, which in turn operates a large pulley *18'*, secured to a shaft *18*, journaled in bearings in 55 hangers, one of which is shown at *19*, depending from the under side of the base *1'*. The shaft *18* has thereon in this case a worm *22*, in mesh with a worm-gear *23*, loosely mounted on a shaft *25*, and bearing at one end 60 against a fixed cheek, while at the other end it coöperates with one member *24* of a coupling device, preferably a friction-coupling, the other element of which may be carried by the worm-gear *23*, as illustrated at *23'*, 65 suitable adjusting and check nuts, such as *26* and *26'*, being employed to secure the proper coupling action. The shaft *25* is journaled in bearings *27* and *27'* at opposite ends of the frame and has thereon a pair of cams, such as *25'* and *25''*, for the purpose of controlling, 70 respectively, the oscillating and feed movement of the blank-carrying means. The blank-carrier *B''* may be operated from the main driving-shaft *15* at a rapid rate of speed by means of a link movement, 75 preferably of such a type as to permit the oscillatory movement of the blank to be varied during the type-forming operation. Here said shaft *15* carries a crank-pin *15''*, which operates a link *30*, pivoted to an oscillatory 80 guide *31*, which in turn is pivoted at a suitable point on the frame and has a guideway *31'*, in which a block *31''* is mounted for sliding movement, said block having pivoted thereto a link *32*, the pivot *32'* of which, in 85 the normal position thereof, is coincident with the center of oscillation of the guide *31*, the other end of said link being pivoted on a rod *33*, carried by the oscillatory blank-carrier *B''* and movable in unison therewith, said 90 link being preferably guided in some suitable manner, as by means of a pair of guide-arms, one of which is shown at *34*. Near the center thereof the link *32* has in this case another link *35* pivoted thereto, the link *35* being in turn pivoted at its lower end to a forked arm, such as *36*, straddling the shaft *25* and guided at its lower end in some suitable manner, as by a pin *37*, said forked arm *36* having thereon an antifriction-roll *36'*, 100 which lies against the face of the cam *25'*, and by means of which said forked arm is raised and lowered to shift the link *32* and the block *31''*, by means of which the angular movement of the center *32'* of the link *32* 105 is varied and the oscillatory movement of the blank-carrier *B''* correspondingly modified. This movement of the center *32'* may be such as to vary the angle of oscillation of the blank-carrier *B''* and hence of the blank *b* from zero to about six degrees at each side of the center movement, as indicated by the lines *19* and *19'* in Fig. 8. A suitable spring, such as *38*, should, of course, be employed for returning the forked arm *36* to its normal 110 position, and said spring may also serve to shift the block *31''* back to its dead-center position and to lower both of the blank-carriers *B'* and *B''*. For the purpose of raising the blank during 115 the oscillation thereof I prefer to make use of one or more wedges, such as *w*, which may be interposed between the carriage *B* and the vertically-movable carrier *B'*, which latter in this case has an inclined face *40* coöperating with a corresponding face *41* of the wedge *w*. This wedge preferably derives its movement from the cam *25''* on the shaft *25*, through connections similar to those by 120 means of which movement is transmitted to 125 130

the link 32, that is to say, in this case a forked arm 42 straddles the shaft 25 and carries an antifriction-roll 42' coöperating with said cam 25'', said forked arm being 5 pivoted at its upper end to a link 43, which in turn is pivoted to an angle-arm 44', secured to a shaft 44, journaled in suitable bearings, (not shown,) said shaft having splined thereon in this case a cam 45, which 10 is preferably guided by the wedge *w* so as to move therewith in the direction of the longitudinal feed of the blank while permitting the wedge to move transversely to such longitudinal feed movement for the purpose of 15 feeding the blank toward the die. Said wedge preferably has an antifriction-roll 46 thereon coöperating with the cam 45 and is forked at its rear end to straddle the shaft 44. Suitable springs may be employed for 20 returning the wedge *w* and the forked arm 42 to their normal positions, the latter being operated by a spring 47, while the wedge may be returned by means of a spring 48 working in a slot in the carriage B and secured to a 25 projection or pin 49 depending from said wedge.

For the purpose of preventing the vertical feed movement of the blank-carriers B' and B'' except when it is desired to form a type I 30 provide suitable means for preventing rotation of the shaft 25, the latter having thereon in this case a crank-pin 25''', which may abut against a stop, such as a spring-pressed stop 50, mounted in a suitable opening in the frame and normally projecting into 35 the path of the pin 25''', said stop 50 having, however, a recess 50' through which the pin 25''' may pass when it is desired to release the shaft 25, this latter operation being accomplished by depressing the stop 50 momentarily, as by means of a key 50''.

As the worm-gear 23 is loose on the shaft 25 it will be evident that until the key 50'' is depressed the shaft 15, and the devices for 45 transmitting movement to said worm-gear, will operate idly, as will the link 30 and the oscillatory guide 31 with its shiftable block 31''. Immediately on the depression of said key, however, the shaft 25 begins to rotate, and this operation will continue until the 50 pin 25''' comes in contact with the stop 50 again. During this rotation of the shaft 25 the cam 25' will gradually shift the center 32' of the link 32, and the cam 25'', through the 55 connections to the wedge *w*, will operate the latter toward the left, as seen in Fig. 9. Immediately on the rising of the center 32' the link 32 will, of course, begin to move in a path of gradually-increasing length and will 60 transmit to the blank-carrier B'' an oscillatory movement, the angle of which will also gradually increase until the predetermined maximum movement is obtained, when the 65 angle of oscillation may be reduced to any desired rate dependent upon the shape of the

face of the cam 25'. During this time, as the wedge *w* raises the two blank-carriers B' and B'', of course the center of oscillation of the latter blank-carrier will be gradually raised, it being preferable to raise said carriers to such an extent that at the end of the type-forming operation the axis of oscillation of the trunnions 3 will be substantially in the face of the finished type, it being understood, of course, that on the completion 75 of the latter the spring 48 will serve to shift the wedge *w* to the right as seen in Fig. 9 and permit the lowering of the blank-carriers B' and B'' by the spring 38.

It should be understood that the mechanism herein described is simply one means for rolling a type-blank or typebar-blank into a type-die at a rate of speed sufficient to increase the molecular action in the mass of metal being operated upon to the point 85 where the heat developed will increase the ductility of such metal, preferably to the point of softening the same, without effecting any change in the physical condition of the portion of the blank that is not being 90 worked. Either the blank-carrier or the die-carrier may, of course, be oscillated rapidly to produce the desired result, and either of these members may be fed toward the other during the formation of the type to permit 95 the gradual working of the same to its finished form. Here the entire work of forming the type is accomplished by oscillating and feeding the blank, and the die-carrier is brought to its proper position and located 100 therein before the die comes in contact with the blank.

The type-forming operation will be effected ordinarily by means of a die substantially of the construction shown herein, although other types of dies may be used to accomplish the same result.

A special advantage of employing a die of the construction shown in the drawings is that it permits the confinement of a given portion of the type-bar blank endwise thereof by a body which operates as a single mechanical part, and indeed is actually constructed in one piece, although it has many functions that might be carried out by a 110 large number of tools each having a single function. The principal feature of construction that distinguishes the die employed herein from other type-dies is the employment in connection with the die proper of a 115 blade or fin at one or both sides of the die for the purpose of compressing and displacing a narrow strip of the stock at one or both sides of the point where a type is to be made, and thereby confining endwise of the blank the 120 portion of the stock to be operated upon at any given time for the formation of a type.

The type-dies shown herein have two blades each, one of them being designated by 5 and the other by 5', and as these blades are 130

somewhat thin the notches made by them in the edge of the typebar-blank will be somewhat narrow, as will the strips of material forced out thereby. These blades form a means for confining between them endwise of the bar the material within any given type-field, but as there are no corresponding end walls on the die to check the flowage during compression the material will, of course, be free to flow out crosswise of the bar. Each of the blades 5 and 5' projects, usually throughout its whole length, beyond the outer wall or bottom wall 6 of its die, and hence throughout the whole period during which a type is being formed these blades serve to confine between them the mass of material that is being shaped. The bottom 6 of the die serves to roll out sidewise the major portion of the material not required for the making of a type. The end walls of the die-space, which are indicated herein by 6', intersect the bottom 6 in the usual way, as at 6", and the edge 6" serves to shear or cut away from the mass of the bar a type-block or type-blank containing sufficient material to fill the die-space and form a finished type; and that part of the edge of the typebar-blank which is operated upon, but is not compressed by the blades 5 and 5', and is not contained within the die-space, is obviously compressed by the bottom wall 6 of the die and is rolled off sidewise of the typebar-blank, but is always confined endwise of the bar by the die-blades just mentioned. Hence none of this surplus material is operated upon in such a manner as to force it into the field of an adjacent type, but instead all of the excess, whether it is forced out by the edges of the blades or by the bottom wall 6 of the die, flows sidewise of the blank and may afterward be severed from the bar to bring the sides of the latter into parallelism with each other.

The manner in which and the extent to which the type-formative material confined between the die-blades, and also supported at its forward side by adjoining stock in advance thereof, is operated upon are dependent upon the oscillation of the blank and also upon the feed movement thereof. Usually a somewhat rapid feed movement will be imparted to the blank during the early stages of the oscillation thereof in order that the type may be roughed out rapidly and afterward finished somewhat more slowly as the work approaches completion. Moreover the center 32' may be shifted away from its normal position to secure the maximum angle of oscillation of the blank B" some time before the type is completely formed and may be returned to such normal position immediately before the upward feed movement of the two blank-carriers B' and B" ceases, but no arbitrary relation between the oscillatory movement of the blank and its upward feed

movement need be maintained provided that the rate of oscillation is sufficiently rapid to produce not only a rolling, a forging, and a swaging action upon the type-blank, but also a mechanical disturbance of the particles of the mass sufficient to heat up and soften the latter, when the die will also operate to mold the softened metal into shape on the hard bar with which it retains its connection and which forms a resistant medium for opposing the compressing action of the die upon the metal and preventing the carrying down of such compressing action any considerable distance into the harder metal below and outside of the die-space. 80

The operations to which the material of the blank is subjected are such as will result in forming a type without impairing the strength of such type-formative material. It has been stated before that these blanks 85 will be suitable composition of type-metal, and moreover they may be either separate typebar-blanks or a continuous strip or ribbon of metal from which the type-bars may be severed after being completed. In 90 every case, however, wrought-metal blanks formed ordinarily by the usual rolling operations should be employed, as I have found in practice that cast-metal blanks are undesirable for the purpose and are not so well 95 adapted to be brought into shape by such operations as are employed in this process. The principal reason for this is that cast metal when rolled and forged in this manner tends to crush and crumble beneath the die 100 instead of compressing and flowing properly, and hence the cast metal will not fill the dies so well as the wrought metal, nor form the smooth faces and sharp edges that the latter will, nor will it maintain its integral connection with the body of the blank without impairment of the strength of the metal even when the heat developed in the metal increases the ductility of the latter to the softening point and the type is partially 110 formed by molding. The manner in which the metal acts when operated upon by the die will, of course, depend very materially upon the composition thereof, and I have found in practice that the best results are secured by operating substantially in the manner described upon wrought-metal blanks composed of tin, antimony, and copper united in such proportions as to give the greatest strength with toughness and sufficient ductility to prevent crumbling and assure flowage of the metal under the action of a die. 115

In forming a type from a cold-metal blank in the manner hereinbefore described it will be evident that the face of the blank will be 125 swaged to a considerable extent shortly after the rolling action begins, this swaging being performed by the face or inner wall of the die; that the rolling will be accomplished chiefly by the base or outer wall of the die 130

and by the edges of the die-blades; that the forging of the type body will be effected principally by means of the end walls of the die, which will usually be considerably inclined in order that the type may be shaped properly and sufficient room left between such walls and the corresponding sides of the type to assure the filling of the die-space during the final stages of the type-making operation; and that the molding of the surface of the type will be effected when the blank is oscillated with sufficient rapidity to soften the mass being operated upon and render it plastic. This heating up of the mass as a result of the rapid mechanical working of the same in contact with the die may be varied considerably, and during the final stages of the operation the shaping of the metal may be accomplished by an operation which is substantially analogous to hot forging; whereas after the operation proceeds so far as to soften the metal and render it substantially plastic the die action will be more nearly analogous to a molding operation.

In carrying out the operation of forming a type according to my present process, as the blank is swung toward the right and toward the left alternately and is simultaneously fed toward the die, the stock at the base of the type-blank or type-block *t* is forged first at one side and then at the other, the forging action being, of course, greatest near the base of the type-block because this part of the type-block is farthest from the axis of oscillation. The forging action, however, extends up the entire length of the side being operated upon and results in a thorough compacting or condensing of the particles of the blank. The forging action being greatest at the base of the type-block the latter will be strengthened most in the region of its base, but the strengthened base will also be connected with the face of the type by a thick layer of condensed metal thoroughly compacted by the forging operation. At the same time that this metal is compressed by the forging action of the end walls *6'* of the die-space the central portion of the type-blank is forced upward into the die, owing to the resistance opposed to the forging action by the inner opposite walls *8* and *8'* of the die space, the upper portion or head of the type-block being forced up farther and farther as the operation proceeds until the metal completely fills the die-space. During this period the cutting edge *6''* of the die shears into the metal of the typebar-blank and gradually completes the cutting out of the type-block or type-blank from the mass of the metal. This type-blank, it will be seen, is not completely sheared from the typebar-blank until the actual completion of the making of the type. In other words, the shearing of the typebar-blank and the formation

of a type from that type-blank are substantially coincident when my improved process is carried out in the manner just described. Each time that a feed movement and an oscillation occur an additional portion of the surplus material confined between the die-blades *5* and *5'* is forced out sidewise of the blank both by the lower edges of these blades and by the bottom wall *6*. After such portion of the surplus has been forced out sidewise in this manner the cutting edge *6''* at the next operation shears farther into the body of the blank, and this action continues until the type is finished. During the final stages of the operation when the metal of the blank becomes plastic as a result of the heat developed therein the die will operate substantially as a means for molding the face of the type to its finished form. Of course when the blank is withdrawn from the die it should be lowered in a straight line in order to avoid injuring the finished type.

After any one type has been formed on the typebar-blank another may be shaped in substantially the same way, as is clearly shown in Fig. 4, but in every case the blade or fin *5* should be so located as to lie close to the side of the next adjacent finished type in order that the types when finished may be sufficiently close to one another. It will be understood, of course, that the blank will be fed to a new position by turning the feed-screw *20* the proper amount and resetting the die-wheel, if necessary, to bring another die to the working position.

The fins *f* and *f'*, which are rolled off from the sides of the bar by the bottom wall of the die and by the edges of the blades *5* and *5'*, respectively, (chiefly by the surfaces *6* and *5'*,) may be removed at any proper time and in any suitable manner, a pair of cutting tools, such as *c*, being shown for the purpose, these preferably operating after a series of types has been formed.

It should be understood, of course, that the spaces between groups of letters or words may be formed in any suitable way, but preferably by means of blank dies, (not shown,) which will roll the metal off in substantially the manner just described. These blank spaces may be of any suitable width, and the letters themselves will be of varying widths, but in all cases it is desirable to form between the words spaces of such width as to make typebars of uniform lengths, whether the blank spaces be of the same width or of different widths, thus assuring the formation of typebars having the types thereon properly spaced.

Having described my invention, I claim—

1. That improvement in the art of making typebars which consists in applying a die to each of the successive type portions along the edge of the blank in succession and rapidly and repeatedly moving said die at each type

forming operation in a direction generally crosswise of the blank and working the portion of metal acted upon by the die at a sufficiently rapid speed to decrease the natural molecular cohesion of the metal in said portion and thereby induce free flowage thereof.

2. That improvement in the art of making typebars which consists in bringing a die into working engagement with each of the successive type portions along the edge of the typebar in succession in a reciprocatory rolling

working movement transversely of the blank and working the portion of metal acted upon and inducing molecular movement therein at a sufficiently rapid rate of speed to generate 15 heat and thereby decrease the natural molecular cohesion of the metal in such portion and thereby induce freer flowage thereof.

FRANCIS H. RICHARDS.

Witnesses:

FRED. J. DOLE,  
C. E. Voss.